

## 1

3,311,512

METHOD OF PRODUCING STEEL STRAPPING  
August F. Mohri and John F. Jarrell, Hamilton, Ontario,  
and Robert C. Reynolds, Burlington, Ontario, Canada,  
assignors to The Steel Company of Canada, Limited,  
Hamilton, Ontario, Canada, a Canadian company  
No Drawing. Filed Apr. 2, 1964, Ser. No. 356,950  
Claims priority, application Canada, Mar. 17, 1964,  
898,040

6 Claims. (Cl. 148—12.1)

This invention relates to a method of producing high tensile steel strapping and the product produced thereby. It is particularly directed to the production of high tensile steel strapping from a silicon semi-killed steel or a capped steel having from about 0.24% to about 0.30% carbon and from about 1.35% to about 1.65% manganese.

Heretofore, high tensile steel strapping commonly has been produced by treating carbon steels having a carbon content of from about 0.45% to about 0.55% and a manganese content of from about 0.60% to about 0.90% by cold reducing the steel to the desired gauge, slitting the cold-reduced steel longitudinally into a plurality of strips of the desired width, feeding the cold-reduced strips continuously into a furnace for heating the strips to a temperature above the critical range and passing the strips into a lead bath held at a predetermined temperature to promote the development of the final desired grain structure and physical characteristics as a result of isothermal transformation.

A disadvantage inherent in this method of producing steel strapping is the requirement for expansive heat treating equipment such as furnaces designed especially to heat treat the cold-rolled steel.

It is, therefore, an important object of the present invention to provide a method of producing high-strength steel strapping which obviates the need for expensive heat treating equipment and permits the production of high strength steel strapping using stress relieving equipment readily available in conventional steel mills.

It is another important object of the present invention to produce steel strapping having the desired properties of strength and ductility from a semi-killed or capped steel.

Another important object of the present invention is the provision of a simple and inexpensive method for the production of steel strapping.

These and other objects of the present invention, and the manner in which they can be attained, will become apparent from the following detailed description of the method of the invention.

We have found that the strength and ductility requirements of a high strength steel strapping can be obtained by means of the present invention from a semi-killed steel having from about 0.01% to about 0.05% silicon or a capped steel having a minor residual silicon content, each having a carbon content of from about 0.24% to about 0.30% and a manganese content of from about 1.35% to about 1.65%, the optimum results being obtained when the carbon content is 0.27% and the manganese content is 1.50%.

Hot rolled steel strip in the form of coils having this metallurgical composition are cold worked by rolling or the like means and reduced about 60% to about 70% in thickness to provide a steel strip having a thickness of from 18 to 23 gauge United States Standard or the like desired gauge thickness. The cold-reduced steel is then stress relieved by process annealing at a temperature of from about 850° F. to about 950° F., preferably at about 900° F., in a controlled neutral or slightly reducing atmosphere for about 6 hours. The steel is then cooled in the neutral or slightly reducing atmosphere to about

## 2

atmospheric temperature and slit longitudinally to provide the narrow strapping strips of a desired width such as  $\frac{3}{8}$ ",  $\frac{3}{4}$ ",  $1\frac{1}{4}$ " and 2" widths from the original full width coil strip. If it is preferred to provide a predetermined degree of surface texture or smoothness to the strapping the strip can be temper rolled or skin passed prior to the slitting step.

The stress relieving of the steel at this temperature results in partial recrystallization or grain alteration of the crystalline structure of the deformed steel to provide the required steel ductility and other physical characteristics while retaining the desired tensile strength. For example, steel strapping according to the present invention  $1\frac{1}{4}$ " in width and about 20 gauge in thickness has a breaking load of 5200 pounds and an elongation of from about 8% to about 10% in six inches.

The present invention provides a number of important advantages. High strength standard and heavy-duty steel strapping having the desired ductility and other physical properties necessary for utilization in banding or otherwise strapping cartons, boxes and the like objects can be produced from a steel of a specific metallurgical composition without the need for the expensive heat treating equipment heretofore necessary. The steel strapping thus can be readily and inexpensively produced in conventional steel mills employing standard low-temperature process annealing equipment.

It will be understood, of course, that modifications can be made in the preferred embodiment of the invention described and illustrated herein without departing from the scope and purview of the invention as defined by the appended claims.

What we claim as new and desire to protect by Letters Patent of the United States is:

1. The method of producing high tensile steel which comprises the steps of cold working a steel having from about 0.24% to about 0.30% carbon and from about 1.35% to about 1.65% manganese to reduce the thickness about 60% to about 70% such that the said steel attains the desired gauge thickness, annealing said steel at a temperature between about 850° F. to about 950 F. for about 6 hours to obtain the desired grain structure and ductility, and cooling the steel to atmospheric temperature.

2. The method of producing high tensile steel strapping which comprises the steps of cold working a strip of steel having from about 0.24% to about 0.30% carbon and from about 1.35 to about 1.65% manganese to reduce the thickness of the strip about 60% to about 70% such that the said strip attains the desired gauge thickness, heating the cold-reduced strip to and maintaining said strip at a temperature between about 850° F. to about 950° F. for about 6 hours to obtain the desired grain structure and ductility, and cooling the strip to atmospheric temperature.

3. The method of producing high tensile steel which comprises the steps of cold rolling a steel strip having a carbon content of about 0.27% and a manganese content of about 1.50% about 60% to about 70% in thickness such that the said steel strip attains the desired gauge thickness, annealing the cold rolled steel strip at a temperature of about 900° F. for about 6 hours to obtain the desired grain structure and ductility, and cooling the strip in a protective atmosphere to atmospheric temperatures.

4. The method of producing high tensile steel strapping which comprises the steps of cold working a steel strip having a carbon content of about 0.27% and a manganese content of about 1.50% to reduce the strip about 60% to about 70% in thickness such that the said steel strip attains the desired gauge thickness, anneal-

ing the cold worked steel strip at a temperature of about 900° F. for about 6 hours to obtain the desired grain structure and ductility, cooling the strip in a protective atmosphere to a temperature below about 200° F., and slitting that strip into relatively narrow strips of a desired width. 5

5. The method as claimed in claim 2 in which the cooled strip is slit into relatively narrow strips of desired width.

6. A high tensile steel strapping produced according to 10 the method claimed in claim 2.

**References Cited by the Examiner****UNITED STATES PATENTS**

2,864,607 12/1958 Renkin ----- 266—3

**OTHER REFERENCES**

Metals Handbook, 1948, Am. Soc. for Metals, pages 354—355.

DAVID L. RECK, *Primary Examiner.*

H. F. SAITO, *Assistant Examiner.*